

H. D. TIEMANN.

PROCESS OF RAPIDLY DRYING TIMBER AND OTHER MOISTURE BEARING SUBSTANCES.

APPLICATION FILED JULY 1, 1909.

942,150.

Patented Dec. 7, 1909.



Witnesses

Fred Bradford  
Thomas G. Shearman.

Inventor  
HARRY D. TIEMANN.

by  
Geo. P. McCauley  
Attorney

# UNITED STATES PATENT OFFICE.

HARRY D. TIEMANN, OF NEW HAVEN, CONNECTICUT.

## PROCESS OF RAPIDLY DRYING TIMBER AND OTHER MOISTURE-BEARING SUBSTANCES.

942,150.

Specification of Letters Patent.

Patented Dec. 7, 1909.

Application filed July 1, 1909. Serial No. 505,454.

DEDICATED TO THE PUBLIC.

*To all whom it may concern:*

Be it known that I, HARRY D. TIEMANN, a citizen of the United States, and an employee of the Forest Service, Department of Agriculture, a legal resident of the State of Connecticut, residing at New Haven, county of New Haven, Connecticut, (whose post-office address is Yale Forest School,) have invented new and useful Improvements in the Process of Rapidly Drying Timber and other Moisture-Bearing Substances, and have made application by petition of even date herewith, under the act of March 3, 1883, chapter 143, 22 Stat., 625, praying that Letters Patent therefor may be granted to me.

The invention herein described and claimed may be used by the Government of the United States or any of its officers or employees in the prosecution of work for the United States or by any person in the United States without payment of any royalty thereon.

The following is a specification of the said invention:

The invention relates to an improvement in the art of rapid artificial drying of wood or other moisture bearing substances and depends upon a specific combination and sequence of operations substantially as described below.

The apparatus does not form an essential part of this invention, my claim of originality being in the combination and sequence of operations. This consists essentially of first heating the wood to be dried in a closed vessel by means of a circulation of, or in the presence of, carbon dioxid ( $CO_2$ ), or other nonoxidizing gas or gases, mixed with a certain amount of water vapor, which amount should at first be as much as the space can contain, and as the wood becomes drier, it should be approximately proportional to the degree of moisture in the wood, as hereafter explained, and when the wood has become thoroughly heated through to the center, cooling it in the same gas from which the water vapor has been removed by condensation, and finally in repeating this operation until the desired degree of dryness has been reached. This whole operation may be conducted at-atmospheric pressure, thus doing away with the expense of heavy apparatus, or at higher pressure

requiring a pressure cylinder. To conduct these operations, the wood is placed in a suitable chamber with non-conducting walls and approximately air-tight. It should be so piled as to allow of free circulation of gas between and around each piece. The wood may be run into the chamber on trucks. The gas, previously heated is then passed into this chamber through distributing plates or pipes, so that it will be uniformly distributed and not impinge directly onto the wood, and the exhaust openings should be similarly arranged. When the air has been displaced, the exhaust gas may be reheated and used over again, thus forming a complete circuit. A certain amount of water vapor is mixed with the heated gas before it enters the chamber, in order to prevent evaporation from the wood during the heating process. If the wood is very wet this will be unnecessary since enough vapor will be supplied by the water in the wood to partially saturate the gas. In partially dry wood, however, the gas should be partially saturated with vapor to a degree approximately corresponding to the degree of dryness of the wood. It should not be enough to cause condensation on the wood.

The temperature of the wood itself, which at first will be less than that of the surrounding gas, is determined by means of a recording pyrometer, with a flexible bulb, the recording dial being outside of the chamber, and the bulb placed in contact with the wood. When the wood has remained in this condition long enough to become uniformly heated clear through to the center (requiring about an hour for partially dry wood one inch thick, or half an hour for wet wood, and longer times according to the thickness), the entering gas is then cooled and at the same time the water vapor removed therefrom by condensation, thus a circulation of cold, dry gas is maintained in place of the hot moist gas, until the wood has become cooled throughout. When heated under pressure greater than atmospheric, the pressure should be reduced during the cooling. The effect of this is that the moisture in the wood is evaporated by the heat of the wood itself. When the wood has cooled, the operation is again gone through with, using less vapor mixed with the heating gas. This is repeated until the desired degree

of dryness is obtained. The degree of vapor present with the gas should correspond approximately to the degree of moisture in the wood.

- 5 The duration of each process depends upon the species of wood, its moisture condition, its dimensions and degree to which it is heated, and the pressure of the gas used. Each operation may require from less than 10 one hour to several hours. If conducted under pressure less time is required. In the absence of air or moisture wood may be heated to a much higher temperature without injury, than when either air or moisture 15 is present. In fact a temperature may be used which would totally destroy the wood for useful purposes if in contact with air or moisture. For example, spruce may be safely heated to 170° C. or even higher under these circumstances.

The principles upon which these operations are based may be briefly described as follows:

- (1) The wood is heated by means of the 25 circulating gas and not by radiation from the walls or from heating coils. Thus the inner parts of the stack of wood are heated as well as the outer part, resulting in the most uniform heating which it is possible 30 to obtain. The greater the pressure of the gas, the more rapid the heating.
- (2) Evaporation during the heating process is prevented by means of the amount of water vapor mixed with the gas. This is 35 a vital point, since evaporation during heating of a piece of wood must necessarily be most rapid at the surface, where it receives the heat, thus causing case hardening and unequal shrinkage. With a very wet piece 40 of wood, this does not apply at first, since considerable evaporation of the free water may take place before any shrinkage begins, and the danger of checking does not occur until the wood begins to shrink.
- 45 Shrinkage begins in most woods when at a moisture content of from 25 to 30 per cent. of the dry weight.

- (3) By cooling the wood in gas free from water vapor or in a vacuum, evaporation 50 takes place and is caused by the heat contained within the wood itself. As the amount evaporated is proportional to the loss in temperature, it follows that the tendency is for evaporation to take place from 55 the interior of the block as much as from the surface, for as soon as evaporation begins at the surface, that portion is cooled and the action checked, whereas it continues from the warmer interior portion of the 60 block. The action is thus self regulating, and the result is as near a uniform evaporation throughout the block clear to the center as it is possible to obtain. It is the unequal drying which causes internal strains

due to unequal shrinkage and these internal strains cause checking, honey combing, warping, and other harmful effects. While it may be impossible to avoid all internal strains absolutely, this process of drying by uniform evaporation throughout the block, 70 reduces them to a minimum. Case-hardening is prevented by this method, if rightly conducted.

(4) Treating the wood in the absence of oxygen overcomes oxidation at high temperatures.

(5) When the wood has cooled to the temperature of the surrounding gas, evaporation practically ceases, and the total amount of water which has evaporated depends upon 80 the temperature to which the wood was heated. In practice it is economy of time not to wait until the wood has completely cooled to the lower temperature.

(6) In order to remove the remaining 85 moisture, the entire operation is again gone through with, and this is repeated until the desired degree of dryness is attained. The wood can be rendered absolutely dry by this means, but in most cases a reduction to 3 or 90 4 per cent. of the dry weight is all that is desirable. Ordinary air dried wood contains about 12 per cent. of moisture.

As the wood becomes drier the temperature to which the wood is raised may be increased with beneficial results. As has been said, spruce, for instance, may be heated to 170° C. The results of this combination and sequence of treatments are (1) Drying 95 wood more rapidly without injury than has heretofore been possible. (2) The product is rendered less hygroscopic by the high 100 temperatures, when again exposed to the outside air. That is to say, its moisture content is less and changes less with changes of humidity of the air, than is the case of air-dried wood. (3) The strength is increased on account of the reduction in moisture. (4) Warping, working, shrinking and 105 swelling are reduced, for the same reason. (5) The resonant quality so much desired in 110 musical instruments is increased.

It is to be understood that while speaking of "wood" in the above description, the process is applicable to other moisture-bearing substances, and I desire my Letters Patent to cover the use of this method for drying all such materials.

The accompanying drawing represents a 120 section at about the middle of the kiln or "closed vessel," Q, referred to in the specification. At top and bottom is an air space running the length of the kiln and separated from the interior by the distributing gratings E and E'. The shaded portions represent 125 impermeable walls of concrete or other such material. The exit flue, O, is at either end of the air space just beneath the roof.

Circulation is maintained by a fan, X, which may be cut off and replaced by a direct gravity circulation by turning a damper in a flue at K. Gas from the fan, X, passes first through the humidifier, H, a box containing water maintained at the proper temperature, as ascertained by the thermometer, C. It then passes under the floor, G, of the kiln through a number of openings at M; thence around the heating coil, N, and up through the distributing grating, E; thence through the pile of lumber, P, and out through the grating, E', to the roof, where it passes through the flue O; thence down through the condensing coil, and back into the fan X. The gas is dried to the desired degree, or humidified to the proper amount, according to the temperatures of the condensing coil, T, and the water bath of the humidifier, H, respectively. The degree of heat in the kiln, Q, is controlled by the heating coil, N, and the temperature of the wood recorded by the autographic thermometer, D, the bulb, D', of which is placed among the lumber.

Non-oxidizing gas is supplied through pipe R on the entering side of the fan X.

Tight canvas and sliding wood or metal doors are used at the ends of the kiln.

A and B are pipe thermometers; F and F' are rollers.

I claim:

1. In the process of drying wood and other moisture-bearing substances, an improvement consisting in the combination and sequence of the following operations: heating the substance by means of a non-oxidizing gas or gases mixed with a certain amount of water vapor until the substance is uniformly or nearly uniformly heated throughout, then followed by cooling in the presence of or by means of the same or other gas or gases containing less water vapor, and repeating this same said sequence of operations until the desired effect and degree of dryness are obtained.

2. In the process of drying wood and other moisture-bearing substances, an im-

provement consisting in the combination and sequence of the following operations: 50 heating the substance by means of a non-oxidizing gas or gases at or near atmospheric pressure mixed with a certain amount of water vapor, until the substance is thoroughly heated through, then followed 55 by cooling at or near atmospheric pressure by means of or in the presence of the same or other gas or gases containing less water vapor, and repeating this same said sequence of operations until the desired effect 60 and degree of dryness are obtained.

3. In the process of drying wood and other moisture-bearing substances, an improvement consisting in the combination and sequence of the following operations:— 65 heating the substance by means of a non-oxidizing gas or gases mixed with a certain amount of water vapor at pressure greater than atmospheric until the substance is thoroughly heated through, then followed 70 by cooling at reduced pressure by means of or in the presence of the same or other gas or gases containing less water vapor, and repeating this same said sequence of operations until the desired effect and degree of 75 dryness are obtained.

4. In the process of drying wood and other moisture-bearing substances, an improvement consisting in the combination and sequence of the following operations: 80 heating the substance by means of a non-oxidizing gas or gases mixed with a certain amount of water vapor until the substance is uniformly or nearly uniformly heated throughout, then followed by cooling in the 85 presence of or by means of the same or other gas or gases containing less water vapor, and repeating this said sequence of operations and increasing the temperature to which the substance is heated as the substance approaches dryness, until the desired 90 effect and degree of dryness is obtained.

HARRY D. TIEMANN.

Witnesses:

H. E. MCKENZIE,  
W. D. BRUSH.